

## UNITED STATES PATENT OFFICE

2,304,925

## PHOTOGRAPHIC DEVELOPER

Edwin E. Jelley, Rochester, N. Y., assignor to  
Eastman Kodak Company, Rochester, N. Y., a  
corporation of New Jersey

No Drawing. Application November 15, 1940,  
Serial No. 365,787

6 Claims. (Cl. 95—88)

This invention relates to photographic developers and particularly to developers for producing colored photographic images.

The methods for forming colored photographic images by coupling development are divided into two classes, namely those in which the color forming or coupling component is incorporated in the emulsion layer prior to exposure and those in which it is dissolved in developing solution. Among the methods in which the coupler is incorporated in the emulsion layer, one type was described in Mannes and Godowsky U. S. application Serial No. 314,689, filed January 19, 1940. According to the process of that application, a coupler is mixed with a cellulosic material and the mixture is dispersed in gelatin in the form of minute particles. Sensitive silver halide grains may be incorporated either in the particles of cellulosic material in coupler or in gelatin in the form of the usual silver halide emulsions.

It has been found that when couplers are incorporated in gelatin layers in this manner in certain cases a very weak color or no color at all is produced when the emulsion is exposed in the usual manner and developed with the customary type of color producing developer.

It is, therefore, an object of the present invention to provide a coupling developer suitable for the development of emulsion layers in which the coupler is rendered non-diffusing by admixture with cellulosic or other particles. A further object is to provide a novel coupling developer for the development of colored photographic images. Other objects will appear from the following description of my invention.

These objects are accomplished by adding to the developing solution of an aromatic alcohol having a relatively low solubility in water, in which the aromatic nucleus is separated by one or more methylene groups from the hydroxyl radical. Such alcohols are powerful solvents for ionized molecules such as the reaction products resulting from the action of exposed silver halide on a color developer. They are also efficient plasticizers for cellulose esters such as cellulose nitrate and for natural gums.

Suitable aromatic alcohols for use in developers according to my invention are the following:

Benzyl alcohol



$\beta$ -phenyl ethyl alcohol



5  $\gamma$ -phenyl-n-propyl alcohol



10 The concentration of the aromatic alcohol should not exceed about 50% of its solubility in the developer used. Benzyl alcohol is soluble in water to the extent of about 40 grams per liter and  $\beta$ -phenylethyl alcohol is soluble in water to the extent of about 16 grams per liter. The amounts used in the developing solution should, accordingly, be kept within the solubility limits.

15 Suitable developers for use with the photographic elements described in Mannes and Godowsky application Serial No. 314,689 are the following:

20 Example 1

|                                             |       |      |
|---------------------------------------------|-------|------|
| 2-amino-5-diethylaminotoluene hydrochloride | grams | 1.0  |
| Sodium sulphite                             | do    | 5.0  |
| 25 Sodium carbonate                         | do    | 30.0 |
| Potassium thiocyanate                       | do    | 0.5  |
| Benzyl alcohol                              | do    | 10.0 |
| Water to                                    | liter | 1.0  |

30 Example 2

|                                             |       |      |
|---------------------------------------------|-------|------|
| 2-amino-5-diethylaminotoluene hydrochloride | grams | 1.0  |
| Sodium sulphite                             | do    | 5.0  |
| 35 Sodium carbonate                         | do    | 30.0 |
| Potassium thiocyanate                       | do    | 0.5  |
| $\beta$ -Phenylethyl alcohol                | do    | 5.0  |
| Water to                                    | liter | 1.0  |

40 Example 3

|                                      |       |      |
|--------------------------------------|-------|------|
| p-amino-dimethylaniline sulphate     | grams | 1.0  |
| Sodium sulphite                      | do    | 2.0  |
| Potassium carbonate                  | do    | 35.0 |
| Potassium thiocyanate                | do    | 0.5  |
| 45 $\gamma$ -Phenyl-n-propyl alcohol | do    | 2.0  |
| Water to                             | liter | 1.0  |

50 It has also been found that aromatic alcohols according to my invention are of value for incorporation in coupler developers in which the coupler is incorporated in the developing solution. When used with developers of this type, there is a great increase in dye density particularly in the denser regions of the scale. This action may be due to the effect of the phenyl alkyl alcohols in aiding penetration of the developer

and coupler through the shell of the dye which forms around the silver halide crystals as they develop, although I do not wish to be limited to this explanation of the action of the agents used according to my invention. I have found that the addition of about 1% of benzyl alcohol, 0.5% of  $\beta$ -phenylethyl alcohol or 0.2% of  $\gamma$ -phenyl-n-propyl alcohol to coupler developers containing dissolved couplers produce this beneficial result. The following example illustrates a developer of 10 this type.

*Example 4*

*Solution A:*

|                                |       |     |
|--------------------------------|-------|-----|
| p-Aminodimethylaniline sulfate | grams | 1   |
| Sodium sulfite                 | do    | 2   |
| Sodium carbonate               | do    | 30  |
| Potassium thiocyanate          | do    | 0.5 |
| Benzyl alcohol                 | do    | 10  |
| Water to                       | cc.   | 900 |

*Solution B:*

|                         |       |     |
|-------------------------|-------|-----|
| 4-nitroacetoacetanilide | grams | 2.5 |
| Isopropyl alcohol       | cc.   | 100 |

(In use, B is added to A.)

The aromatic alcohols proposed according to my invention may also be used in the development of colored images in which couplers are rendered non-diffusing in gelatin layers by reason of molecular size or attached to the gelatin and in which couplers are rendered non-diffusing by incorporation in other than cellulose esters such as synthetic resins, natural gums or the oil formers described in Jelley and Vittum application Serial No. 371,612, filed December 26, 1940. They may also be incorporated in black and white developers. The developers of Examples 1, 2 and 3 will produce black and white images in the absence of a coupler in the emulsion layer.

It will be understood that the couplers or color formers used to produce the dye images to which this invention principally relates are

of the well known type containing a phenolic hydroxyl or reactive methylene group which produce dye images in the presence of the oxidation product of primary aromatic amino coupling developing agents.

My invention is to be considered as limited only by the scope of the appended claims.

I claim:

1. A photographic developer comprising a silver halide developing agent and an aromatic alcohol having the following formula:



where  $x$  is a positive integer of from 1 to 3.

2. A photographic color developer comprising a primary aromatic amino developing agent and an aromatic alcohol having the following formula:



where  $x$  is a positive integer of from 1 to 3.

3. A photographic color developer comprising a primary aromatic amino developing agent and an appreciable amount, not in excess of 50% of its solubility in the developer, of an aromatic alcohol having the following formula:



where  $x$  is a positive integer of from 1 to 3.

4. A photographic color developer comprising a primary aromatic amino developing agent and a small amount of benzyl alcohol.

5. A photographic color developer comprising a primary aromatic amino developing agent and a small amount of  $\beta$ -phenyl ethyl alcohol.

6. A photographic color developer comprising a primary aromatic amino developing agent and a small amount of  $\gamma$ -phenyl-n-propyl alcohol.

EDWIN E. JELLEY.